

May 4, 1926.

1,583,495

H. M. SCHLEICHER

## METHOD OF REFINING LEAD

Filed Nov. 6, 1925

Fig. I



Fig. 2



Fig. 3.



INVENTOR  
Henry M. Schleicher  
BY  
Pennie Davis Hamm & Edmunds  
ATTORNEYS

Patented May 4, 1926.

1,583,495

# UNITED STATES PATENT OFFICE.

HENRY M. SCHLEICHER, OF MONTERREY, MEXICO, ASSIGNOR TO AMERICAN METAL COMPANY, LTD., OF NEW YORK, N. Y., A CORPORATION OF NEW YORK.

## METHOD OF REFINING LEAD.

Application filed November 6, 1925. Serial No. 67,223.

To all whom it may concern:

Be it known that I, HENRY M. SCHLEICHER, a citizen of the United States, residing at Monterrey, Nueva Leon, Mexico, have invented certain new and useful Improvements in Methods of Refining Lead; and I do hereby declare the following to be a full, clear, and exact description of the invention, such as will enable others skilled in the art 10 to which it appertains to make and use the same.

This invention relates to a method of refining lead, and particularly to the removal of elements such as arsenic, antimony, tin 15 and zinc therefrom.

The refining of lead has been accomplished heretofore by subjecting it while in a molten condition to oxidation in the presence of an alkali metal hydroxide and 20 an oxidizing agent such as the oxygen of the atmosphere or oxidizing salts. The method depends upon the selective oxidation of impurities, usually arsenic, antimony, tin and zinc, and the absorption 25 of the oxidized elements by the alkali metal hydroxide. The operation as conducted heretofore has been carried out in a non-continuous manner, the alkali metal hydroxide being disposed upon the surface of 30 the lead bath, either in a partially immersed cylinder or otherwise and permitted to remain until it has absorbed the desired proportion of the oxidized impurities. When 35 the alkali metal hydroxide has absorbed the impurities to the extent which is advisable in view of the subsequent treatment, it is usual to replace it with fresh alkali metal hydroxide and to repeat the operation until 40 the desired purification is accomplished. This point in the operation is hereinafter called "saturation". The method when so conducted is relatively slow because of the necessity for retarding the reaction as the 45 purification approaches the finishing stage either with reference to the saturation of the alkali metal hydroxide or of the depletion of the impurities in the lead. Care must be taken to avoid going too far in either direction. Furthermore, the operation of the 50 method depends upon the oxidation of the lead and the subsequent oxidation of the impurities by the lead oxide. The impure lead oxidizes less readily than lead from which the impurities have been removed substan- 55 tially. Consequently the maximum rate of

removal of the impurities cannot be attained under the conditions mentioned.

It is the object of the invention to provide a method of purifying lead which is more rapid and satisfactory in operation and 60 which is adaptable for continuous operation and the selective separation of several impurities if such are present.

Further objects and advantages of the invention will be apparent as it is better understood by reference to the following specification and to the accompanying drawing in which a suitable type of apparatus for 65 the practice of the method is illustrated diagrammatically. In the drawing, 70

Fig. 1 is a sectional view of a type of apparatus adapted for the removal of a single element or of the several impurities together or in succession;

Fig. 2 is a similar view illustrating the 75 apparatus in which the impurities are removed separately; and

Fig. 3 indicates the arrangement of the apparatus for counter-current operation.

In starting the refining operation I employ instead of a bath of the impure lead, one from which the impurities have been removed. This ensures the most active oxidation and facilitates the removal of the impurities from the lead which is added 80 continuously to the bath. Thus, as a simple example of the operation, the lead in the bath may contain less than .01% of antimony if no silver is present, or about .01% of antimony if the lead is to be desilverized 85 subsequently. It is assumed for the purpose of simplifying the explanation that arsenic, tin and zirc are absent. To this bath the impure lead, containing a considerably larger proportion of antimony, is fed 90 continuously at a rate corresponding to the rate of removal of the antimony therefrom. At the same time a corresponding amount of the purified lead is withdrawn continuously and preferably from the bottom of 100 the bath. For this purpose the vessel in which the lead bath is maintained can be provided with a suitable outlet such as a siphon so that a constant quantity of the metal is retained therein. A siphon is preferable because it will draw off the lead from the bottom of the vessel where the purest lead tends to settle in a layer because of its greater specific gravity. 105

The purification is accomplished by the 110

action of a suitable reagent such as an alkali metal hydroxide or a mixture thereof with common salt in the presence of an oxidizing agent. The alkali metal hydroxide or mixture can be disposed so as to contact with the surface of the molten metal and particularly to be engaged by the impure metal which is introduced to the bath. Preferably the impure metal is fed directly to the alkali metal hydroxide or mixture and the molten lead in the bath is circulated by means of a pump so that it passes successively therethrough. The oxidation may be caused by atmospheric air which is blown or otherwise introduced to the bath of molten metal. Alternatively oxidation depends upon the introduction of an oxidizing salt such as an alkali metal nitrate. In the presence of the oxidizing agent the lead is partially oxidized and the lead oxide produced is carried into contact with the impure metal and the alkali metal hydroxide or mixture. The lead oxide oxidizes the impurities in the impure metal and the oxidized impurities are absorbed by the alkali metal hydroxide or mixture so that the impurities are progressively separated and the amount of impurities present in the lead of the bath remains substantially constant. If a single body of the reagent is used it will be necessary to delay the operation when it approaches the finishing stage. By providing two separate bodies of the reagent one can be removed and replaced while the other is being utilized in the continuation of the operation. Alternatively, the reagent can be introduced continuously in the proper proportion to maintain a substantially constant saturation with the impurities at a point where the reaction is active and the corresponding amount of the reagent containing the impurities can be withdrawn continuously.

As the result of the operation as described the impure lead containing antimony is supplied to the bath at a constant rate and the purified lead containing an amount of antimony corresponding to that originally in the bath is removed continuously from the bottom thereof. This permits the refining of the lead to the desired purity rapidly and efficiently, the operation being particularly effective because of the fact that the pure lead oxidizes rapidly, ensuring consequently the necessary amount of lead oxide to remove the impurities from the impure lead which enters the bath. Excessive saturation of the reagent is likewise avoided so that the operation is not delayed during any period.

The invention may be applied to the successive removal of arsenic, antimony, tin and zinc from the lead. These elements can be removed in the same receptacle by maintaining suitable oxidizing conditions

but preferably a series of receptacles are used, each being provided with the necessary reagent and being connected in such a manner that the lead will flow through the receptacles in succession. The receptacles will be filled in initiating the operation with lead containing only the impurities which are intended to remain therein at the termination of the purification in that receptacle. Thus, for example, in the first receptacle the lead will contain antimony and tin but no arsenic. The second will contain antimony but no tin or arsenic and the third a minimum amount of antimony. In conducting the operation the impure lead is fed to the first receptacle, and after purification therein it flows into the second receptacle and finally into the third where the purification is completed. If desired the necessary reagent and the oxidizing material are fed to each of the receptacles and a corresponding amount of the impure reagent can be withdrawn from these receptacles, thus permitting operation in a continuous manner. It is obvious that the rate of removal of the several impurities will vary, and in operating with successive receptacles as indicated the rate of flow of the metal must be adjusted to the rate of elimination of the impurity which is removed most slowly. The rate of oxidation in the other receptacles is then adjusted to ensure removal of the respective impurities.

In purifying hard lead, that is, lead containing antimony which should not be removed, the method of operating would involve the provision of two or more baths of antimony and lead, each with provision for the introduction of the necessary reagent and oxidizing material. Impure hard lead and the fresh reagent are continuously added in such a manner as to permit countercurrent passage through the system, that is to say, the lead flows in one direction while the reagent flows in the other. In this case the alkali metal nitrate or other oxidizing agent is introduced to the system only at the place where the fresh reagent is added. Any antimony which is oxidized and absorbed by the reagent tends to be reduced again by the other impurities in the successive receptacles and thus reenters the lead. The same procedure can be employed also with advantage when the lead contains a single impurity which is to be removed or where two or more impurities are removed in a single operation.

Referring to Fig. 1 of the drawing, a kettle 5 may be supported in a suitable furnace to permit the maintenance of the lead bath 6 contained therein at the required temperature. A receiver 7 is supported so that its lower edge is beneath the surface of the bath of molten metal, the receiver being

adapted to contain the reagent 8 which rests upon the surface of the lead bath and is thus prevented from escaping. A pump 9 of any suitable kind adapted to handle the molten metal is disposed beneath the surface of the bath and is provided with a delivery pipe 10 through which the metal is fed to the receiver so that it falls through the reagent therein. Fresh reagent can be supplied 10 through a conduit 11. A siphon 12 is arranged to withdraw metal from the lower part of the bath and to deliver it to a suitable receptacle 13. The lead originally present in the kettle 5 should, as above indicated, have the composition of the desired product, being free, for example, from arsenic and tin and having the minimum proportion of antimony. The impure lead containing the antimony to be removed is introduced at the desired rate through a conduit 14 to the reagent 8, and if desired a supply of the reagent can be introduced similarly through the conduit 11. If the reagent is supplied continuously an overflow 15 permits the continuous withdrawal of a portion of the reagent containing the impurities. The reagent used may be an alkali metal hydroxide or a mixture thereof with common salt (sodium chloride) with or without the addition of an oxidizing agent such as an alkali metal nitrate. Various other chemical compounds and mixtures thereof can be utilized for the purpose of the invention. Air can be introduced to the bath by any suitable means. As the operation proceeds a portion of the relatively pure lead in the bath is oxidized and the lead oxide in turn oxidizes the impurities present in the lead which is fed continuously to the bath. The reagent absorbs these oxidized impurities. If the reagent is supplied continuously it can be maintained at the desired concentration with respect to the impurities by the continuous withdrawal of a portion of the reagent. Otherwise it is desirable to employ two or more bodies of the reagent, one of which is operative while the other is being removed.

In Fig. 2 of the drawing a series of kettles 16, 17 and 18 are adapted to be maintained at the desired temperature by suitable furnaces provided for that purpose. Lead is withdrawn from the kettle 16 through a siphon 19 provided for that purpose and is delivered to the kettle 17 and the lead, after treatment in the kettle 17, is delivered through a siphon 20 to the kettle 18. It is finally withdrawn through a siphon 21 into a receptacle 22 which is provided to receive the purified metal. Each of the kettles is provided with a receiver 23 for the reagent and a pump 24 in each of the kettles forces the molten metal upwardly through a pipe 25 and into the receiver. The impure lead is delivered to the receiver in the kettle 16 by a conduit 26 and passes through the several kettles in succession as indicated. Fresh reagent can be added to the receivers in each of the kettles or it can be added to the receiver in the last kettle and conveyed thereafter through the other receivers successively. As an example of the operation arsenic can be removed in the kettle 16, tin in the kettle 17 and antimony in the kettle 18. In starting the operation the lead in each of the kettles should have the composition with respect to impurities which is to be attained by purification therein. Thus the lead in the kettle 18 will contain the minimum amount of antimony and lead having this composition can be withdrawn continuously from this kettle.

In Fig. 3 of the drawing the arrangement of the kettles for counter-current operation is indicated. The kettles 27, 28 and 29 may be disposed in the relation indicated with receivers 30 therein to hold the reagent. The fresh reagent is introduced to the receiver 30 in the kettle 27 and the impure lead is introduced to the receiver 30 in the kettle 29. The purified lead is withdrawn then from the kettle 27 and the reagent saturated with the impurities is withdrawn from the receiver 30 in the kettle 29. The molten lead and the reagent are transferred between the kettles and receivers therein in the manner indicated by the arrows so that these materials travel in counter-current relation. It is to be understood, of course, that each of the kettles is provided with a pump to circulate the molten metal and that siphons or other means may be employed to transfer the metal and the reagent as required.

The reagent recovered from any of the operations as described contains the impurities originally present in the lead and these impurities constitute valuable products. The reagent can be treated suitably for the recovery of the several impurities, the operation being so conducted as to regenerate alkali metal hydroxide or other material employed, as the reagent.

From the foregoing description the principles of the operation of the method will be understood. The efficiency of the method depends upon the more rapid oxidation which is accomplished under the conditions mentioned and the maintenance of the reagent at such a concentration with reference to the several impurities that the most effective absorption thereof is assured. While the operation is conducted preferably as hereinbefore indicated, the principles thereof may be applied in a variety of ways depending upon the nature and proportion of the impurities which are present in the lead. The absence of one or more of the impurities mentioned will obviate the necessity of the particular step involved in its removal. Similarly the rate at which the lead is permitted to flow

through the apparatus and the oxidizing conditions mentioned must be varied in accordance with the proportion of that impurity which is removed least rapidly by the purifying operation. Likewise various changes can be made in the apparatus employed without departing from the invention or sacrificing any of the advantages thereof.

I claim:

10 1. The method of refining lead, which comprises maintaining a bath of molten lead, which is substantially free from the substance removed as impurities, in contact with a reagent capable of absorbing the oxidized impurities and in the presence of an oxidizing agent, and adding lead containing impurities to be removed to the bath at substantially the rate of absorption of the oxidized impurities by the reagent.

20 2. The method of refining lead, which comprises maintaining a bath of molten lead, which is substantially free from the substance removed as impurities, in contact with a reagent capable of absorbing the oxidized impurities and in the presence of an oxidizing agent, adding lead containing impurities to be removed to the bath at substantially the rate of absorption of the oxidized impurities by the reagent and withdrawing the purified lead from the bath at an equivalent rate.

30 3. The method of refining lead, which comprises maintaining a bath of molten lead, which is substantially free from the substance removed as impurities, in contact with a reagent capable of absorbing the oxidized impurities and in the presence of an oxidizing agent, adding lead containing impurities to be removed to the bath at substantially the rate of absorption of the oxidized impurities by the reagent and supplying the reagent so as to maintain a substantially constant concentration of the impurities therein.

40 4. The method of refining lead, which comprises maintaining a bath of molten lead, which is substantially free from the substance removed as impurities, in contact with a reagent capable of absorbing the oxidized impurities and in the presence of an oxidizing agent, adding lead containing impurities to be removed to the bath at substantially the rate of absorption of the oxidized impurities by the reagent, supplying the reagent so as to maintain a substantially constant concentration of the impurities therein and withdrawing a portion of the reagent containing the impurities.

50 5. The method of refining lead, which comprises maintaining a bath of molten lead, which is substantially free from the substance removed as impurities, in contact with a reagent capable of absorbing the oxidized impurities and in the presence of an oxidizing agent, adding lead containing impuri-

ties to be removed to the bath at substantially the rate of absorption of the oxidized impurities by the reagent and circulating the molten lead through the reagent.

6. The method of refining lead, which comprises maintaining a bath of molten lead, which is substantially free from the substance removed as impurities, in contact with a reagent capable of absorbing the oxidized impurities and in the presence of an oxidizing agent, adding lead containing impurities to be removed to the bath at substantially the rate of absorption of the oxidized impurities, circulating the molten lead through the reagent and withdrawing the purified lead from the bath in proportion to the amount of impure lead added thereto.

7. The method of refining lead, which comprises maintaining a bath of molten lead, which is substantially free from the substance removed as impurities, in contact with a reagent capable of absorbing the oxidized impurities and in the presence of an oxidizing agent, adding lead containing impurities to be removed to the bath at substantially the rate of absorption of the oxidized impurities, circulating the molten lead through the reagent, withdrawing the purified lead from the bath in proportion to the amount of impure lead added thereto and supplying the reagent so as to maintain a substantially constant concentration of the impurities therein.

8. The method of refining lead, which comprises maintaining a bath of molten lead, which is substantially free from the substance removed as impurities, in contact with a reagent capable of absorbing the oxidized impurities and in the presence of an oxidizing agent, adding lead containing impurities to be removed to the bath at substantially the rate of absorption of the oxidized impurities, circulating the molten lead through the reagent, withdrawing the purified lead from the bath in proportion to the amount of impure lead added thereto, supplying the reagent so as to maintain a substantially constant concentration of the impurities therein and withdrawing a portion of the reagent containing the impurities.

9. The method of refining lead, which comprises maintaining a series of baths of molten lead, each of which is substantially free from the substance removed as impurities in the respective bath, in contact with a reagent capable of absorbing the oxidized impurities and in the presence of an oxidizing agent, adding lead containing impurities to be removed to the first bath of the series and conveying the lead progressively through the series of baths.

10. The method of refining lead, which comprises maintaining a series of baths of molten lead, each of which is substantially free from the substance removed as impuri-

- ties in the respective bath, in contact with a reagent capable of absorbing the oxidized impurities and in the presence of an oxidizing agent, adding lead containing impurities to be removed to the first bath of the series, conveying the lead progressively through the series of baths and supplying the reagent so as to maintain a substantially constant concentration of the impurities therein.
- 10 11. The method of refining lead, which comprises maintaining a series of baths of molten lead, each of which is substantially free from the substance removed as impurities in the respective bath, in contact with a reagent capable of absorbing the oxidized impurities and in the presence of an oxidizing agent, adding lead containing impurities to be removed to the first bath of the series, conveying the lead progressively through the series of baths, supplying fresh reagent to the last bath of the series and conveying it progressively through the preceding baths in counter-current relation with the lead.
12. The method of refining lead, which comprises maintaining a series of baths of molten lead, each of which is substantially free from the substance removed as impurities in the respective bath, in contact with a reagent capable of absorbing the oxidized impurities and in the presence of an oxidizing agent, adding lead containing impurities to be removed to the first bath of the series, circulating the lead through the reagent in each bath, and conveying the lead progressively through the series of baths.
13. The method of refining lead, which comprises maintaining a series of baths of molten lead, each of which is substantially free from the substance removed as impurities in the respective bath, in contact with a reagent capable of absorbing the oxidized impurities and in the presence of an oxidizing agent, adding lead containing impurities to be removed to the first bath of the series, circulating the lead through the reagent in each bath, conveying the lead progressively through the series of baths and supplying the reagent so as to maintain a substantially constant concentration of the impurities therein.
14. The method of refining lead, which comprises maintaining a series of baths of molten lead, each of which is substantially free from the substance removed as impurities in the respective bath, in contact with a reagent capable of absorbing the oxidized impurities and in the presence of an oxidizing agent, adding lead containing impurities to be removed to the first bath of the series, circulating the lead through the reagent in each bath, conveying the lead progressively through the series of baths and supplying the reagent so as to maintain a substantially constant concentration of the impurities therein.
15. The method of refining lead, which comprises maintaining a bath of molten lead containing impurities in the proportion desired in the final product, continuously adding impure lead to the bath and withdrawing the product therefrom and removing the impurities to the desired degree by circulating the lead in contact with a reagent capable of absorbing the oxidized impurities in the presence of an oxidizing agent.

In testimony whereof I affix my signature.

HENRY M. SCHLEICHER.